

# UNITED STATES PATENT OFFICE.

GEORGE LANZENDORFER, OF BRAINTREE, MASSACHUSETTS.

## METHOD OF PREPARING SHAPED FIBERS.

1,193,703.

Specification of Letters Patent.

Patented Aug. 8, 1916.

No Drawing.

Application filed July 21, 1913. Serial No. 720,315.

To all whom it may concern:

Be it known that I, GEORGE LANZENDORFER, a citizen of the United States, a resident of and whose post-office address is Braintree, 5 county of Norfolk, and State of Massachusetts, have invented an Improvement in Methods of Preparing Shaped Fibers, of which the following description, in connection with the accompanying drawings, is a 10 specification, like characters on the drawings representing like parts.

This invention relates to shaped fibers and the method of producing the same.

In order that the principle of the invention 15 may readily be understood, I shall describe one embodiment of the product and the best modes known to me for producing the same.

An important purpose of my invention is 20 to shape or fashion fibers to any desired form and preferably to curl the same so that they may be used for upholstery work and other purposes.

In producing the described product I 25 preferably employ structural fibers especially those of the monocotyledonous class. Among such fibers I may enumerate manila, sisal, istle, hemp, palm leaf fibers, the fibers from bromelia and aloe plants, from bamboo and rattan, and the cocoanut and the tilandsia fibers or southern moss.

The ultimate product of my invention is a 30 mass of tangled fibers each of which is shrunk into a permanent form which is preferably a curl. I may secure this product in 35 several modes, but I prefer to treat the fibers in groups such as bundles or strands instead of individually treating them, as the latter procedure involves a more extended period 40 of manipulation and hence is more costly. Any of the said modes is, however, within the scope of my invention.

In accordance with one method of practising my invention, I arrange any of the 45 fibers previously referred to, or any suitable mixture of them, in bundles or strands around a suitable form or mandrel so as to impart thereto a shape which determines the final set thereof. Or, if desired, the fibers 50 may be twisted into single bundles or strands, or two or more of such bundles or strands can be twisted together so that the twist thus imparted will determine the final form or set of the fibers. In the event that 55 two or more of the bundles or strands are twisted together, it will be evident that the

fibers of each bundle or strand constitute a former for the fibers of the other strands, thus avoiding the necessity of providing a rod or bar former toward which the fibers 60 are wound.

I will first describe one method of practising my invention wherein the fibers, of whatever nature, are twisted into rope form, in which case the individual fibers have imparted thereto a curled or spiral set. In accordance with this method the fibers are by any well known mechanical means made into a sliver or strand which may be twisted upon itself or two or more of these slivers 65 may be twisted together into a rope. In the event that two or more slivers are twisted together, the fibers of each sliver will act as a former for the fibers of the other sliver or slivers. This twisting of the material 70 into rope form imparts a certain curl to the fibers but such curl is not permanent. In order to render the curl or set permanent the rope is treated with some suitable shrinking agent until it is thoroughly impregnated 75

thereby. Any suitable shrinking agent may be employed, such, for example, as any of the caustic alkalis, such as soda, potash and the like, or any suitable acid such as sulfuric acid. The well known mercerizing 80 process is well adapted for this purpose, the mercerizing agent commonly employed being caustic soda. The fibers shrink considerably under the action of the agent. The rope is then subjected to a washing process 85 to remove as much as possible of the agent and then is thoroughly dried. The single fibers have thus imparted thereto a final set which is the form they have assumed in the twisted strand or rope. After the rope is 90 dried I, by a reverse mechanical operation, untwist the strands and pick or separate out the fibers individually. Each of these fibers has now a permanent spiral-like curled form.

The fibers are then assembled in a tangled 95 mass and may be used for upholstery or other purposes. The product of my invention may also be obtained by treating the fibers in the loose state as they come from the bale or package with a suitable shrinking agent, such, for example, as caustic soda solution. The fibers are then washed to remove the shrinking agent and are then twisted 100 into rope form either in a wet state or after drying the same. If the fibers are 105 dried before being twisted into rope form the rope should be thoroughly wetted and

- the subsequent drying will impart to the fibers thereof the curled shape or set to which I have referred. The twisted rope is then untwisted in any suitable manner so as 5 to separate the fibers individually. At any suitable stage of the process, but preferably after the treatment of the material with the shrinking agent, such operations as dyeing or sizing may be carried out.
- 10 Having thus described one illustrative embodiment of my invention, I desire it to be understood that although specific terms are employed, they are used in a generic and descriptive sense and not for the purposes of 15 limitation, the scope of the invention being set forth in the following claims.
- Claims:
1. That method of imparting a permanent set to fibers which consists of twisting 20 a mass of fibers together, impregnating the mass with a mercerizing agent, washing and drying the mass, and then reversing the twisting operation to separate the individual fibers.
  - 25 2. That method of imparting a permanent set to fibers which consists of grouping the fibers into a plurality of slivers or strands, twisting said slivers into a rope,

impregnating the rope with caustic soda, 30 washing and drying the rope and then reversing the twisting operation to separate the individual fibers.

3. That method of imparting a permanent set to fibers which consists in treating 35 them in a loose state with a shrinking agent, washing the fibers, twisting a mass of the fibers together and permitting them to set, and finally separating the mass into its constituent fibers.

4. That method of imparting a permanent set of fibers which consists in grouping the fibers into a plurality of slivers or strands, twisting said slivers together into a rope, so that the fibers of each sliver constitute a former for the fibers of the other sliver or slivers, impregnating the rope with a shrinking agent and then untwisting the rope into its constituent twisted fibers.

In testimony whereof, I have signed my name to this specification, in the presence of 50 two subscribing witnesses.

GEORGE LANZENDORFER.

Witnesses:

JOHN R. MOULTON,  
IRVING U. TOWNSEND.

Copies of this patent may be obtained for five cents each, by addressing the "Commissioner of Patents, Washington, D. C."